

Dec. 6, 1932.

A. T. COLWELL

1,889,916

METHOD OF MAKING COMPOSITE VALVES

Filed May 20, 1931

FIG. 1



FIG. 2



FIG. 3



FIG. 4



FIG. 5



FIG. 6

INVENTOR  
Archie T. Colwell

Charles J. Gillen

627

775

## UNITED STATES PATENT OFFICE

ARCHIE T. COLWELL, OF CLEVELAND, OHIO, ASSIGNOR TO THOMPSON PRODUCTS, INCORPORATED, OF CLEVELAND, OHIO, A CORPORATION OF OHIO

## METHOD OF MAKING COMPOSITE VALVES

Application filed May 20, 1931. Serial No. 538,787.

This invention relates to a method of sealing hollow metallic articles and in particular to a method of sealing the chambers in metal cooled valves.

It is an object of the present invention to provide a method of sealing the head of a valve which is provided with a heat conducting insert from the hot gases of the exhaust chamber.

It is a further object of this invention to provide a simple and expedient method of sealing an aperture in a metal body by puddling metal in the aperture.

Other and further important objects of this invention will be apparent from the disclosures in the specification and the accompanying drawing.

This invention (in a preferred form) is illustrated in the drawing and hereinafter more fully described.

*On the drawing*

Figure 1 is a cross-sectional view of a recess blank used in making a valve according to my invention.

Figure 2 is a cross-sectional view of the blank of Figure 1 showing a metallic insert in the recess thereof.

Figures 3, 4 and 5 illustrate steps in the carrying out of my process.

Figure 6 is a cross-sectional view of a valve formed in accordance with my invention.

*As shown on the drawing*

In carrying out this invention, a suitable blank 1 of tungsten steel, nickle-chromium steel or other suitable valve material is formed by forging or cutting a slug from rolled stock. The blank 1 is recessed at 2. The recess 2 is preferably cylindrical and concentric with the blank 1. The recess 2 extends through one end of the blank and for a considerable distance therein.

A plug 3 of copper, aluminum or similar metal having a relatively high rate of heat conductivity is inserted in the recess 2. The blank 1 may be heated to expand the recess 2 before receiving the plug 3 or both the blank 1 and insert 3 may be cold. It is also to be

understood that the insert 3 may be melted and poured into recess 2.

The composite blank thus formed from the blank 1 and insert 3 is then forged by any suitable method, such as extruding. In this operation, a head 5 and a stem 6 are formed on the blank. The metal of insert 3 is drawn out to form the core 7 in the stem and a portion thereof is spread out into the head as shown at 8. This operation leaves a recess 60 or aperture 9 in the head 5 which in the ordinary course of the extruding process is filled with the insert metal. This metal is removed from the aperture 9 by any suitable method as by drilling. Molten metal 11, preferably 65 of the same composition as the metal of the valve blank, is then poured into the aperture 9 and allowed to unite with the metal of the head 5. Excess metal 11 is scraped from the top of the valve. 70

The partially formed valve is then re-forged and machined to obtain the finished product. In this last operation, pressure is applied to the head 5 and metal 11 to firmly bond them. As a result, the head 12 of the 75 finished valve presents a homogeneous appearance.

A valve formed by this method is shown in Figure 6. The valve comprises a head 12, a stem 13, the stem having a core 14 of a heat 80 conducting metal therein. A portion of the metal core 14 is spread out in the head as shown at 15. Such a valve is particularly useful in high speed engines where it is necessary to draw the heat from the head of the 85 valve.

In such operation, it has been found that the sealed head formed by my method remains firmly bonded under the most severe operating conditions. 90

It will be seen that I have provided a method of making a valve which is simple and expedient, which does not require any machinery other than is necessary in ordinary valve making and which will form a valve capable of withstanding the severe conditions of use in high pressure, high speed automotive engines. 95

I am aware that many changes may be made and numerous details of construction may be 100

varied through a wide range without departing from the principles of this invention, and I, therefore, do not purpose limiting the patent granted hereon otherwise than necessitated by the prior art.

5 I claim as my invention:

1. The method of making a metal cooled valve, which comprises partially filling a recessed blank with a metal having a relatively high rate of heat conductivity, forging the blank, puddling a molten metal into the opening of the recess and reforging the valve.

10 2. The method of making a metal cooled valve which comprises forging a metal blank containing an insert of softer metal, replacing part of the softer metal by a hard metal and reforging to incorporate the hard metal into the valve.

15 3. The method of making a metal cooled valve which comprises forging a metal blank containing an insert of a metal of relatively high rate of heat conductivity to provide a partially finished valve having a core of said insert metal extending through the head thereof, removing a portion of said core, filling the recess thus formed with molten metal of the same composition as that of the blank and reforging the blank to form a finished valve.

20 4. The method of sealing a recess in the head end of a valve having a soft metal insert extending through part of the head portion which comprises puddling a molten metal in the recess and reforging the valve.

25 5. In testimony whereof I have hereunto subscribed my name at Cleveland, Cuyahoga County, Ohio.

ARCHIE T. COLWELL.

40

45

50

55

60

65